

Dec. 6, 1938.

G. M. ALLEN ET AL

2,139,568

SPINNERET AND METHOD OF PRODUCING THE SAME

Filed Jan. 7, 1937



INVENTORS  
GEORGE M. ALLEN  
GILBERT C. BARTON  
BY THEIR ATTORNEYS

*Howson and Howson*

## UNITED STATES PATENT OFFICE

2,139,568

SPINNERET AND METHOD OF PRODUCING  
THE SAME

George M. Allen, Swarthmore, and Gilbert C. Barton, Chester, Pa., assignors, by mesne assignments, to American Viscose Corporation, a corporation of Delaware

Application January 7, 1937, Serial No. 119,488

4 Claims. (Cl. 76—107)

This invention relates to spinnerets and methods of producing the same, and more particularly to spinnerets or jets adapted to be connected to a spinning pump for spinning rayon or the like by squirting or extruding spinning solution through minute holes in the face of the spinneret.

In the viscose process and some other processes of spinning rayon it is necessary to have the spinneret made of a material resistant to both acids and alkalis. For this reason the spinneret up to the present time has usually been made of the noble metals. In view of the thousands of such spinnerets both in use and in stock which are necessary for the operation of a commercial rayon spinning plant, the amount of metal required represents a large capital investment. It is therefore the main object of the present invention to reduce the quantity of metal required for the construction of the spinneret.

The diameter of the face, diameter of flange, and height of spinneret are constants determined by usage.

The face of the spinneret must not only withstand the internal pressure of the spinning solution but at various times the external pressure of a man's thumb endeavoring to wipe the face clean. Further, the operator presses his thumb against the majority of the holes so as to increase the internal pressure to such an extent that the rate of flow will be increased, thereby dislodging any dirt particles in the free holes.

The flange of the spinneret must be of sufficient thickness to retain its corrugated contour under compression. As the seal of the spinning solution is made at this point, a thinning of the metal in this area was not deemed advisable.

The side wall of the spinneret is subject only to tension stresses of the spinning pressure. As this area constitutes 60% of the total weight of the spinneret, it is therefore a particular object of this invention to reduce the thickness of the side wall of the spinneret. A further object is to increase the tensile strength of the side wall by work hardening, simultaneously with the thinning, by a swaging operation.

Other objects will be apparent from the following description in connection with the accompanying drawing, in which—

Figure 1 is a vertical cross-section through a blank or piece of metal in the early stage of the manufacture of the spinneret, also showing in dotted lines the condition after the side walls have been thinned and lengthened by a swaging operation;

Figure 2 is a vertical cross-section through the spinneret shell according to the present invention; and

Figure 3 is a face view or end elevation illustrative of one form of swaging machine by means of which the spinneret shell may be thinned.

The spinneret according to the present invention as shown in Figure 2 comprises a single piece of noble metal formed into a cup shaped shell, having a face 4 formed by the bottom of the cup-shape, and a side wall 5 integral therewith and extending therefrom to an annular flange 6, by means of which the spinneret may be mounted for connection to a spinning pump for spinning rayon or the like.

The flange 6 is annularly corrugated to provide a leak-proof joint when mounting the spinneret, and the face 4 is ultimately tooled to provide the extrusion orifices through which the spinning solution is to be squirted, in the spinning process.

The side wall 5 is materially thinner than the remainder of the shell, being for example of about half the thickness of the face 4 and the flange 6. This thinner side wall is of increased tensile strength to compensate for the reduction to thickness, and to take the tension stresses resulting from the pressure of the spinning pump.

The spinneret described above is manufactured by first forming a cup-shape, preferably by a pressing operation, and then thinning the side wall, preferably by a swaging operation. While the thinning may be done by a spinning operation, swaging is less difficult to control than spinning. In addition either the swaging or spinning operation work hardens the metal. The swaging method being preferred, the manufacture of the spinneret is described in detail according to that method.

A plate or piece of noble metal of uniform thickness is dished or formed into a cup-shape as shown in full lines in Figure 1, for example by a pressing operation. This form has a base 14, an annular flange 16, and a side wall 15 therebetween. The side wall 15 in this stage is of the same thickness as the base 14 and flange 16, but the length thereof constituting the depth of the cup-shape, is materially less than the depth of the finished spinneret.

For the swaging operation, the blank shown in full lines in Figure 1 is mounted on a mandrel 17 having if necessary, a small taper in order to strip the shell from the mandrel. The blank on the mandrel is inserted in a swaging machine and the side wall 15 is subjected to swaging operation, which reduces the thickness thereof to materially

thinner than the thickness of the base 14 and the remainder of the shell. At the same time, the swaging work-hardens the metal and increases the tensile strength at least compensating for the reduction in thickness.

5 One form of swaging machine is illustrated in Figure 3, which comprises a revolving spindle 7 having in its face a diametral slot 8, in which are slidably mounted a set of cooperating swaging dies 9. These dies are held between backers 10 10 slides in the same groove and having rounded ends projecting beyond the periphery of the spindle.

Surrounding the spindle 7 is an annular rack 15 12 loosely containing a plurality of annularly spaced rolls 13. The revolution of the spindle 7 causes the dies and backers to pass between successive pairs of opposing rolls 13 which force the dies 9 together. The dies revolve rapidly around 20 the work, which is stationary, while the rack 12 revolves very slowly, being moved only by the slight motion of the rolls 13 during the time of contact with the backers, but which evenly distributes the effect of the dies.

25 The dies 9 are blocks of hardened steel which have formed on their inner faces the impression of the shape or the diameter of the work it is desired to produce, with an enlargement or flare at the outer or entering end, large enough to allow the 30 unreduced stock to enter. The dies are set up by placing shims (not shown) between the dies 9 and backers 10, which cause the backers to project further outward in the path of the rolls 13. The dies, backers and shims are held in place in the 35 slot 8 by suitable plates (not shown) over the face of the spindle 7.

In swaging the side wall of the spinneret, the 40 smaller the amount of reduction in thickness for one set of dies, the less danger of failure of the metal during that operation, but of course a large number of operations is undesirable. By dividing the total reduction in thickness into steps by four operations with four different sized sets of dies, the swaging may be accomplished, even with grain 45 structure not of the maximum fineness.

We have constructed spinnerets, starting with a metal of a thickness of 15 mils (thousandths of an inch) and reducing the side wall to 8 mils in one swaging operation using one size of swaging 50 die, and from 8 mils to 5 mils by a second swaging operation using a smaller size of swaging die, but we prefer to start with a metal of 10 mils thickness, and reduce the side wall to 5 mils by one operation with one size of die. To accomplish 55 this it is necessary that the metal be of such fine grain structure as to withstand the swaging without rupture or other failure which would increase the amount of expensive scrap.

We prefer to use an alloy of 70% gold and 30% platinum. However other proportions of these metals may be used, or alloys of other noble metals, or even a noble metal alone. It will be understood that many other modifications may be made without departing from the spirit of the invention, within the scope of the appended claims.

We claim:

1. The method of making a shell for a spinneret for use in spinning rayon which comprises forming a cup shape member of less depth than the finished article of noble metal having an integral base portion constituted by the bottom of the cup shape for perforation to permit spinning 10 solution to be extruded therethrough and a side wall, and hammer swaging said side wall and thereby extending it to its finished length while thinning it and increasing its hardness and tensile strength. 15

2. The method of making a shell for a spinneret for use in spinning rayon which comprises forming an integral cup shape member of less depth than the finished article of noble metal having a face portion constituted by the bottom 20 of the cup shape for perforation to permit spinning solution to be extruded therethrough, a side wall and an attachment flange, and hammer swaging said side wall and thereby extending it to its finished length while thinning said side wall 25 and increasing its hardness and tensile strength. 30

3. A shell of noble metal for a spinneret for use in spinning rayon comprising an integral face portion for perforation to permit spinning solution to be extruded therethrough and a side wall, the shell being formed from a cup shape member of noble metal of less depth than the finished article and the side wall of which has been hammer swaged, thereby thinning and extending it to its finished length, the side wall being 35 thinner and of greater hardness and tensile strength than the face portion. 40

4. A shell of noble metal for a spinneret for use in spinning rayon comprising an integral face portion for perforation to permit spinning solution to be extruded therethrough, a side wall, and an attachment flange, the shell being formed from a cup shape member of noble metal of less depth than the finished article and the side wall of which has been hammer swaged, thereby thinning 45 and extending it to its finished length, the side wall being thinner and of greater hardness and tensile strength than the face portion. 50

GEORGE M. ALLEN.  
GILBERT C. BARTON.